

## UNITED STATES PATENT OFFICE

JAMES E. GRAHAM, OF NEWTON, MASSACHUSETTS, ASSIGNOR TO BIRD & SON, INC., OF EAST WALPOLE, MASSACHUSETTS, A CORPORATION OF MASSACHUSETTS

## FLOOR TILE

No Drawing.

Application filed September 3, 1931. Serial No. 560,999.

This invention relates to a floor tile, and particularly to a resilient floor tile having advantages and properties not found in floor tiles heretofore.

5. The invention provides a resilient floor tile that is extremely tough and durable, relatively non-saponifying and non-water absorbent, remarkably resilient to fats, oils, grease and other materials that floors are likely to be subjected to. In addition to these properties, this floor tile has wear resistance not found in other resilient floor tiles, which is further enhanced by the fact that the composition or size of tile does not change on aging. Other 10 resilient tiles, rubber and linoxyn base tiles, are readily subject to aging which renders them hard and brittle, lacking in resilience and toughness as time goes on. This tile is so constituted that when properly made and 15 cured, it will never change until it has worn out; the ingredients of this tile are so chosen and combined that oxidation and moisture have practically no action on the tile. This tile has great utility in that it is not expensive 20 to make or install, may be made in the most attractive colors and patterns, and in any size or design wanted.

All tiles may be differentiated as belonging to one of two classes; resilient and non- 25 resilient. In the former class are included rubber tile, cork tile with an oxidized oil binder, and the so-called linoleum tile which is similar to the cork tile but contains in addition to cork and linoxyn, mineral and other fillers. In the relatively non-resilient tile field may be classed ceramic tile, marble and asphalt tile.

I do not employ any backing or carrying 30 agent for the tile and I confine my invention to a flat tile, and not to a rollable sheet material (with or without a backing) for, by so doing, I am able to make a floor tile that is stronger, tougher and more permanent than a material made up in roll form. The tile is 35 homogeneous in composition, that is, made up of the same composition throughout, which provides a uniform appearance though the tile is worn thin.

In the manufacture of floor tile in accordance 40 with this invention, I employ finely di-

vided materials or fillers of definite degrees of fineness combined with a binder, including as an essential constituent of the binder a cellulose ester, nitrocellulose being preferred for this purpose because of its ability to produce a tough, elastic binder with good cementing or bonding properties and when properly compounded with other materials to be relatively non-saponifying, and resistant to oils, fats, grease, etc. I have found 55 that nitrocellulose must contain a definite amount of true plasticizing agent to make a suitable binder for a tile. I refer to a true plasticizing agent as one in which nitrocellulose is readily soluble, such as tri-cresyl phosphate or dibutyl phthalate, as differentiated from a softening agent, such as castor oil. I have found that castor oil or similar oil softening agent may be washed out of 60 a tile composition and its very presence makes 65 a tile that is easily dirtied on account of the tackiness of the surface produced when softening agents are used.

I employ nitrocellulose of relatively high viscosity 20-200 sec. types (preferably from 50 to 200 seconds), with a nitrogen content of 11-13%. One hundred parts of dry nitrocellulose requires 80 to 110 parts, and preferably 90 to 100 parts, of tri-cresyl phosphate to make a suitable binder for a tile. If more 75 than this amount is used, the tile is too soft for practical application and will indent badly under load. If less than the designated amount of plasticizer is used, the tile is too hard and non-resilient. These limits have 80 been carefully worked out and cannot be disregarded from if a wholly satisfactory tile is to be produced. I have found tri-cresyl phosphate to be the most satisfactory plasticizer 85 for tile as it has greater plasticizing action per unit volume than most plasticizers; it is colorless, fire resistant and permanent.

In conjunction with the nitrocellulose and plasticizer, I use a definite percentage of a resin, such as ester gum, to improve the binding properties of the nitrocellulose without softening or rendering the resulting tile too tacky. I use 20 to 30 parts ester gum to 100 parts of dry nitrocellulose; other resins that are fairly alkali resistant may be used in 90 95 100

place of ester gum. The resin greatly increases the internal bond and assists in making the fillers resistant to moisture and other agents destructive to floor coverings.

5 The nitrocellulose, plasticizer and resin are brought to the consistency of a thick paste in a mixer of the Werner-Phleiderer type by the use of an active solvent such as butyl acetate. I then add to this binder the cork and fillers.

10 I have found that it is practically impossible to make a tile from this composition by sheeting unless cork of a definite degree of fineness is used. Also, if too much coarse cork is used, the tile is rough and dirties very easily; or, if the cork is too fine, the tile will be badly blistered and unsalable. As a preferred example of graded cork (all passing a 40 mesh screen) suitable for use in this floor tile, I give the following:—

|                                                 | Per cent |
|-------------------------------------------------|----------|
| Passing 40 mesh and retained on 48 mesh screen  | 10       |
| Passing 48 mesh and retained on 60 mesh screen  | 15       |
| Passing 60 mesh and retained on 80 mesh screen  | 15       |
| Passing 80 mesh and retained on 100 mesh screen | 10       |
| Passing 100 mesh screen                         | 50       |

25 This table of graded cork has been found to give the right percentage of roughs and fines and makes a tile which is free from blisters, and is smooth and glossy. If more than 50% of the cork passes a 100 mesh screen, the surface of the tile will show blisters and the tile becomes unsightly and unsalable; if less than 50% passes a 100 mesh screen, the tile will have a rough surface that dirties readily.

30 This composition is passed through a sheeting calender and is cut up into tiles of the required sizes and shapes. These tiles must be thoroughly cured and all the volatile solvent got rid of before they are ready for use. This mixture can not be sheeted on a backing of any type; it would cause a flexible backing to curl badly and, in the case of a rigid backing, the composition would show hair line cracks throughout.

35 A typical and preferred composition tile is as follows:—

100 parts 50 to 200 sec. nitrocellulose  
90 parts tricresyl phosphate  
20 parts ester gum  
50 125 parts #40 mesh cork (as described above)  
150 parts clay (amorphous mineral filler)  
150 parts asbestos (fibrous mineral filler)  
55 100 parts "Titanox C"—(titanium dioxide precipitated on a base) coloring pigment.

Additional coloring or pigment as required.

60 This composition will produce a smooth, uniform tile, resistant to indentation, relatively non-saponifiable, unaffected by mild acids, oils, grease, fat, etc. The mineral fillers may be varied as to color, and type of finish wanted, but the proportions of nitro-

cellulose, plasticizer and type of cork used cannot be varied to any appreciable degree and produce a salable tile. By salable tile, I mean a tile free from apparent defects such as roughness, blisters, etc.

70 This application is a continuation in part, insofar as concerns common subject-matter, of my application Ser. No. 386,483, filed August 16, 1929.

75 What I claim is:—

1. A floor tile of homogeneous composition of substantial thickness, said composition including graded cork substantially all passing a 40 mesh screen and a substantial portion of which passes a 100 mesh screen and finely divided mineral materials bonded together by a resin, a cellulose ester having a viscosity of from 50 to 200 seconds, and a plasticizer.

2. A floor tile of homogeneous composition of substantial thickness, said composition including graded cork filler substantially all passing a 40 mesh screen and a substantial portion of which passes a 100 mesh screen, and finely divided mineral materials, a nitro-cellulose bonding agent having a nitrogen content of from 11% to 13% and a viscosity of from 50 to 200 seconds, and a plasticizer.

3. A floor tile of homogeneous composition, said composition including a nitrocellulose bonding agent having a nitrogen content of from 11% to 13% and a viscosity of more than 20 seconds, a plasticizer in an amount equal to at least 80% by weight of said nitrocellulose bonding agent, a resin, a graded cork filler substantially all passing a 40 mesh screen and substantially half passing a 100 mesh screen, amorphous and fibrous finely divided mineral fillers, and pigment.

4. A floor tile of homogeneous composition, said composition including a nitrocellulose bonding agent having a nitrogen content of from 11% to 13% and a viscosity of more than 20 seconds, a plasticizer in an amount equal to at least 80% by weight of said nitrocellulose bonding agent, a resin, a graded cork filler all passing a 40 mesh screen and substantially half passing a 100 mesh screen, finely divided mineral filler, and pigment.

5. A floor tile of homogeneous composition, said composition including a nitrocellulose bonding agent having a nitrogen content of from 11% to 13% and a viscosity of more than 40 seconds, tri-cresyl phosphate in an amount equal to between 90% and 100% by weight of said nitrocellulose bonding agent, a resin, a graded cork filler all passing a 40 mesh screen and substantially half passing a 100 mesh screen, finely divided mineral filler, and coloring matter.

6. A floor tile of homogeneous composition including a nitrocellulose bonding agent having a nitrogen content of from 11% to 13% and a viscosity of more than 20 seconds,

tri-cresyl phosphate in an amount equal to between 80% and 110% by weight of said nitrocellulose bonding agent, a resin, a graded cork filler all passing a 40 mesh screen and substantially half passing a 100 mesh screen, finely divided mineral filler, and coloring matter.

7. A floor tile of homogeneous composition including a nitrocellulose bonding agent having a nitrogen content of from 11% to 13% and a viscosity of more than 20 seconds, tri-cresyl phosphate in an amount equal to between 90% and 100% by weight of said nitrocellulose bonding agent, a resin, a graded cork filler all passing a 40 mesh screen and substantially half passing a 100 mesh screen, finely divided mineral filler, and coloring matter.

JAMES E. GRAHAM.

20

25

30

35

40

45

50

55

60

65